

Jan. 8, 1952

W. A. McMILLAN

2,581,685

## IMPRÉGNATION DE MATERIAUX ABSORBANTS

Filed June 16, 1948



*INVENTOR.*

WALLACE A. McMILLAN

BY

Daniel Shaffer  
J. H. Graham  
**ATTORNEYS**

ATTORNEYS

## UNITED STATES PATENT OFFICE

2,581,685

## IMPREGNATION OF ABSORBENT MATERIAL

Wallace A. McMillan, Glenham, N. Y., assignor  
to The Texas Company, New York, N. Y., a corporation of Delaware

Application June 16, 1948, Serial No. 33,310

9 Claims. (Cl. 117—92)

1

This invention relates to the impregnation and coating of absorbent or fibrous materials with bituminous compositions to saturate and then surface coat the materials to render them waterproof and weather-resistant. More particularly, the invention relates to an improved process for saturating felt with a normally solid asphalt followed by surface coating of the saturated felt with a filled asphalt in the manufacture of asphalt roofing materials, including roll roofing and shingles.

This is a continuation-in-part of my co-pending application, Serial No. 524,499, filed February 29, 1944, and now abandoned.

Roofing felt is very susceptible to the absorption of moisture from the atmosphere. It is well recognized that the moisture content of the felt must be effectively removed in order to obtain the required saturation or impregnation of the felt with asphalt. The percentage of voids filled with asphalt and the percentage saturation of the felt are measures of the extent of moisture removal and asphalt impregnation of the felt in the saturating process, and have a direct bearing on the weather resistant qualities of the finished roofing. Roofing felt, as furnished by the manufacturer, contains a maximum of 5% moisture; but, upon subsequent storage and transportation, particularly under humid atmospheric conditions, the felt absorbs additional moisture until the moisture content may be in equilibrium with that of the atmosphere.

Numerous methods of driving off the moisture from the felt prior to the saturating step have been proposed, such as passing the felt strip or sheet through drying ovens or over steam heated rolls; but in practice these methods add considerably to the cost of the process and do not always achieve the desired end. The general practice in roofing manufacture is to immerse the moisture-containing felt sheet, without previous drying, in a body of hot asphalt maintained at an elevated temperature of the order of 250—450° F., and allow the heat from the asphalt to vaporize the moisture which is driven off in the form of vapor while the felt is simultaneously being impregnated with the molten asphalt. Considerable difficulty due to foaming of the asphalt saturating bath has been experienced in the past with this method, requiring constant vigilance on the part of the operator to prevent the tank from foaming over, and often necessitating reducing the level or depth of molten asphalt in the saturating bath while concomitantly reducing the line speed of the travelling felt sheet. Pro-

posals have heretofore been made to employ certain anti-foam additives, such as stearic acid, in the saturating bath; but such additives as have heretofore been employed have had to be used in such large proportions as to deleteriously affect the properties of the finished roofing, particularly from the standpoint of weatherability.

Following the saturating step, the travelling sheet of asphalt impregnated felt is then given a surface coating of a so-called filled asphalt, which is a mixture of molten normally solid hard asphalt (lower ASTM penetration) with a finely divided filler of the character of pulverized oyster shell, dolomite, and the like. This is accomplished by premixing the filler with the molten asphalt, and then flowing the resultant mix onto the travelling sheet. In practice, it is found that there is considerable air and water vapor entrainment in the highly viscous mix which shows up in the form of substantial vapor bubbles trapped in the surface coating. This affects the uniformity of the coating layer and contributes to poor weatherability and blistering of the product in service.

It is accordingly a principal object of the present invention to overcome the foregoing objections and to provide an improved process of continuous manufacture of asphalt roofing at efficient line speed, and which will insure the maintenance of the desired operating conditions in both the saturating and coating steps over long periods of continuous operation so as to give a product having the improved weatherability heretofore obtained during only short intervals of spotty operation.

Another object of the present invention is to provide an improved combination of the saturating and coating steps to achieve a final product of improved weathering characteristics in uniform, easily maintained, continuous operation.

Still another object of the present invention is to improve the saturating process to uniformly maintain a higher percentage of voids filled with a particular grade of harder roll saturant to insure improved weatherability of the final product.

A further object of the present invention is to also improve the coating step to substantially eliminate the entrainment of vapor bubbles in the surface coating.

Other objects and advantages of the present invention will be apparent from the following description, the attached drawing and the appended claims.

In accordance with the present invention, it

has been found that a very small amount of a liquid organic silicone of the order of about 0.1-10 parts per million by volume based on the asphalt in the saturating bath, not only substantially inhibits foaming of that bath, thus eliminating the danger of overflow even with a high liquid level near the top of the tank, but also provides a felt sheet emerging from that bath which contains a heavier surface film of molten asphalt imparting to the sheet a characteristic shiny wet appearance. By thus maintaining the saturating bath of substantial depth and at a temperature of about 250-450° F., and preferably about 375-425° F., and then withdrawing the impregnated sheet with the substantial surface film and looping the same to allow it to cool, the surface film rapidly dries in to provide a saturated sheet which can uniformly be maintained at a minimum of 85% or higher of voids filled with asphalt, even though the line speed of the felt is increased over that heretofore permissible. In addition, by utilizing a normally solid asphalt having an ASTM penetration (100 grams, 5 seconds) at 77° F. within the range of about 30-60 for the saturating bath, which heretofore has involved increased difficulties in non-uniform operation, the finished product has been found to be uniformly superior from the standpoint of freedom from blistering on atmospheric exposure. In addition, it has also been found that a very small amount of the liquid organic silicone of the order of 0.1-10 parts per million by volume based on the asphalt in the coating mix effectively prevents the permanent entrainment of vapor bubbles in the molten mix when the filler is incorporated therein, so that the ultimate surface coating on the impregnated felt sheet is substantially free from trapped vapor bubbles. The combination of these steps enables a roofing material of high quality and improved weatherability to be uniformly manufactured at high line speed over substantial periods of continuous operation.

The invention is more particularly illustrated in the attached drawing which is a diagrammatic illustration of apparatus for carrying out the improved method.

Referring to the drawing, a roll 10 of dry felt is unwound from the felt reel onto the dry looper indicated at 11. The latter is of conventional construction involving a series of rolls moving in an endless chain at a velocity less than that of the felt, so that the felt is formed into loops between the individual rolls as indicated at 12. The looper acts as a reservoir of felt material permitting flexibility in the feed of the travelling felt strip through the apparatus. From the looper, the felt passes through pairs of guide rolls 13 and 14 into a presaturating section 15 of the saturating tank indicated generally at 16. As shown, the presaturating section 15 is of less depth than the main saturating section 17 of the tank. Each section is equipped with a series of closely spaced upper rollers 18 and a lower series of rollers 19, so that the felt travels over an upper roller, thence downwardly into the molten asphalt and around a lower roller, and then back up to the next upper roller in series, to receive a plurality of immersions while in the form of loops as indicated at 20.

The function of the presaturating section 15 is primarily to eliminate moisture from the felt by contact with the molten asphalt at a temperature above 250° F. and thus well above the vaporization point of the contained moisture. While some impregnation of the travelling felt with as-

phalt occurs in this section, it is purposely designed of rather shallow depth, so that the depth of immersion of the felt is comparatively small, and the liberated water vapor has only a limited distance to travel to reach the surface of the molten asphalt and escape to the atmosphere. Even with this arrangement, considerable difficulty has been encountered in the past due to copious foaming of the saturating bath, with the foam on the surface of the bath often building up to a height of 4 to 5 ft. resulting in overflow from the tank if the level of molten asphalt is not immediately lowered therein. It should be understood that a presaturating section is not essential to the present invention.

The asphalt saturants employed in tank 16 are the blown petroleum asphalts, or the blended asphalts obtained by blending a steam reduced residual or asphaltic stock with a blown asphalt, and which are normally solid at atmospheric temperatures and possess an ASTM penetration (100 grams, 5 seconds) at 77° F. within the range of about 20-125, and an ASTM softening point (ball and ring method) within the range of 100-180° F. As discussed more in detail hereinbelow, the asphalt saturant preferably has an ASTM penetration at 77° F. of about 30-60, since the harder type asphalt saturant has been found to give improved weatherability when manufactured in accordance with the present invention. Also, in accordance with the present invention, the asphalt saturant within tank 16 contains a very small amount of a liquid organic silicone of the order of about 0.1-10 parts per million by volume based on the asphalt in the bath. This has been found to inhibit foaming such that not more than an inch or two of foam is present on the surface of any portion of the bath during long periods of continuous operation, thereby permitting the level of the bath to be uniformly maintained near the top of the saturating tank. For example, in a saturating tank having a total depth of about 7 ft. in the deeper saturating section 17, the level of molten asphalt may conveniently be arranged just below the upper series of rolls 18, providing a depth of immersion in the pre-saturating section 15 of about 2½ ft. and in the main saturating section 17 of about 5½-6 ft. Ordinarily, the amount of the organic silicone employed in the bath will be about one part per million by volume; although it is found that once having dispersed this amount of the organic silicone effectively throughout the saturating bath, its anti-foam properties will be preserved without further addition for a substantial period of running, or until the effective concentration of the organic silicone may drop to about as low as 0.1 part per million. Larger amounts of the organic silicone than about ten parts per million are avoided as unnecessary. Moreover, the larger amounts appear to alter the physical properties of the asphalt and also destroy the glossy surface finish of the felt strip emerging from the last submergence in the saturating section 17 of the bath. As pointed out above, one of the features of the present invention resides in the operation of the saturating step with the proper controlled amount of the organic silicone within the small critical range specified above, together with maintenance of the temperature and depth of the bath, so that the traveling felt sheet is withdrawn from the bath in a condition in which it retains a substantial surface film of molten asphalt thereon, providing a characteristic glossy

wet or shiny appearance, which surface film then rapidly penetrates the withdrawn felt. While the reason for this unusual effect has not been definitely ascertained, it is postulated that the organic silicone, in addition to inhibiting foaming of the bath, also inhibits the accumulation of a retarding or insulating film of water vapor on the surface of the immersed sheet, thereby permitting more rapid penetration of the impregnating asphalt and also enabling a thicker surface film of asphalt to be retained as the sheet is withdrawn from the bath, and then facilitating the rapid penetration of this surface film into the sheet. In addition to the effect on the glossy surface film, the use of larger proportions of the organic silicone also appears undesirable from the standpoints of deleteriously affecting the adhesive properties of the saturated sheet for the subsequent granular coating, as well as affecting the compatibility of the sheet for the subsequent filled coating. Whatever the action may be, it has been found that operation in accordance with the foregoing principles uniformly gives a saturated felt sheet with a minimum of at least 85% voids filled with asphalt and generally in excess of 87% voids filled.

The organic silicones useful for purposes of the present invention include any of the polymeric organic silicon oxide condensation products which have heretofore been proposed as anti-foam agents for certain organic liquids, particularly mineral lubricating oils at normal atmospheric or mildly elevated temperatures (see Trautman et al. No. 2,416,504 and Larsen et al. No. 2,375,007). Structurally, these compounds are composed essentially of a plurality of silicon atoms linked together through oxygen atoms, with each silicon atom having attached to it at least one organic radical, these products also being known as organo-siloxanes. The oily liquid condensation products obtained by polymerization of organo-silane diols (each silicon atom having attached 2 organic radicals), such as, for example, the dimethyl silicone, are particularly advantageous for purposes of the present invention. As is well known, these compounds may be obtained by hydrolyzing a Grignard reaction product of an organic magnesium halide and an ether solution of silicon tetrachloride, followed by evaporation of the ether and condensation or polymerization of the resulting hydrolyzed Grignard reaction product by heat in the presence of air. The condensation process proceeds through a liquid product of lower molecular weight to a solid plastic of higher molecular weight. For purposes of the present invention, the liquid organic silicones which are usually insoluble in heavy oils of the character of mineral lubricating oil are employed. A dimethyl silicone polymer obtained from the Dow-Corning Corporation under the trade name of "Dow-Corning Fluid" has been used with very satisfactory results. This liquid material is marketed in varying viscosities ranging from about 100 to 1,000 centistokes at 77° F. Analyses of representative samples of this material are as follows:

|                                   | A     | B           |
|-----------------------------------|-------|-------------|
| Carbon, per cent by weight.....   | 32.35 | 31.04-31.55 |
| Hydrogen, per cent by weight..... | 8.15  | 7.84-7.98   |
| Silicon, per cent by weight.....  | 36.50 | 35.6-35.7   |
| Oxygen (by difference).....       | 23.00 | 25.14       |
| Approximate mol. wt.....          | 268   | 4500        |

The organic silicone is conveniently incorpo-

rated in the asphalt saturant by first forming a naphtha or kerosene solution thereof, and then incorporating the resulting silicone concentrate in the molten asphalt. For example, a kerosene concentrate containing one part of the silicone to 999 parts by volume of the kerosene is then added in the proportion of 1 cc. of the concentrate to 1,000 cc. of the molten asphalt to give one part per million by volume of the organic silicone dispersed in the asphalt.

The saturated felt sheet withdrawn from the saturating tank 16 with its glossy surface film, as previously described, then passes to a wet looper indicated at 22 where the travelling sheet 15 is formed into a series of loops 23 providing time for cooling. The natural shrinkage of the asphalt, upon cooling, causes the excess surface film of asphalt to be drawn into the felt, thereby resulting in improved saturation.

20 The travelling sheet then passes by guide rolls 24 and 25 to the coating section where a surface coating of filled molten asphalt is applied to both the top and bottom surfaces of the sheet. For this purpose, molten asphalt is fed from storage tank 27 into a suitable mixer or agitator such as the turbomixer indicated at 28, into which the finely divided solid filler, such as ground oyster shell, dolomite and the like, is supplied by the travelling conveyor 29. For example, a suitable coating mix may be composed of about 35-60% by weight of ground oyster shell, and about 65-40% by weight of a hard coating asphalt having an ASTM penetration at 77° F. of about 15-25. The resulting mix from agitator 28 is 30 supplied to the asphalt coating storage tank 30 from which it is fed to the applicators 31 and 32 extending across the top and bottom of the travelling sheet. The coating mix is applied to the travelling sheet at a temperature of about 40 350-400° F., preferably around 385° F., in order to secure satisfactory adhesion of the hard filled coating.

As noted above, considerable difficulty has been experienced in the past due to the entrainment 45 of air and water vapor bubbles in the viscous mix formed in agitator 28. A large proportion of these entrained bubbles persist in the coating mixture held within storage tank 30 and then supplied to the applicators 31 and 32, with the result that the surface coating layers applied to the travelling sheet have a characteristic mottled appearance due to the entrained vapor bubbles. This, of course, affects the uniformity of the coating even though subsequent processing may 55 largely break and eliminate the trapped bubbles.

In accordance with the present invention, this difficulty has been overcome by incorporating in the molten asphalt in supply tank 27 a very small amount of the same type of liquid organic silicone used in the saturating bath. Here again, the proportion of organic silicone used is within the range of 0.1 to 10 parts per million based on the volume of the molten asphalt, and preferably about one part per million. By having the 60 silicone present in the molten asphalt at the time the solid filler is mixed therewith in agitator 28, it has been found that vapor entrainment in the viscous mix is substantially eliminated. The net result is that the surface coating layers applied 65 to the top and bottom of the travelling sheet are essentially free from entrained vapor bubbles, and desired uniformity of the coating across the width of the sheet is assured.

Following the application of the top and bot- 75 tom coating layers, the travelling sheet then

passes through the coating squeeze rolls indicated at 33, which function to regulate the amount of the coating applied and consequently the weight of the sheet. By adjusting the coating squeeze rolls closer together, a larger proportion of the coating layers is removed to decrease the weight of the sheet per unit area; and conversely by separating the squeeze rolls, the weight of the sheet is increased. The travelling sheet is then subjected to finishing operations in a conventional manner. These operations are not illustrated since they form no part of the present invention. Thus, where a mineral surfaced roll roofing or shingle is being manufactured, the mineral particles are applied to the upper surface of the sheet following the squeeze rolls 33. Where a smooth surfaced roll roofing is being made, mineral particles are, of course, not added but a layer of talc is applied. The sheet is then run through a series of press and cooling rolls or drums, thence to a finishing looper where the final cooling for handling takes place, and finally to a roll roofing winder or to the shingle cutter, as the case may be.

The following example is given to illustrate the present invention. During the manufacture of a ninety pound mineral surfaced roll roofing in accordance with the conventional old procedure, it was found that the line could not be operated at a speed of more than 135 ft. per minute, and, moreover, had to be stopped for short intervals in order to prevent the saturator from foaming over. At this time, the depth of molten asphalt in the saturator had been reduced to 2½ ft., and there was a blanket of foam on the surface thereof 4 to 5 ft. deep. One hundred ccs. of a kerosene solution of the dimethyl silicone polymer, prepared by adding one part of the silicone to 999 parts of the kerosene was then added to the saturator in the presaturating section 15 at the point where the felt enters the asphalt; and the foam immediately subsided almost to the saturant level. Eight hundred ccs. of the kerosene-silicone concentrate were additionally added at different points in the saturating tank and in the saturant storage tank (not shown but connected with the saturating tank 16), so that the silicone was distributed, as quickly as possible, throughout the saturator system holding 635 barrels of asphalt, thereby providing one part per million of silicone by volume on the basis of the molten asphalt in the system. Within five minutes after adding the silicone, the line speed was increased to 185 ft. per minute, the saturant level was raised to a point about 18" from the top of the tank, and there was not more than 1" of foam on the surface of the saturant at any point in the tank. Moreover, at the end of the tank where the saturated felt was withdrawn from the saturator, the surface of the molten asphalt was free from bubbles. The withdrawn sheet had a glossy wet appearance which rapidly penetrated into the withdrawn sheet. Production continued at a line speed of 185 ft. per minute without any further difficulty, resulting in increased production by about 35 rolls per hour. It was further observed that the asphalt surface film on the travelling sheet withdrawn from the saturator appeared to dry in more rapidly than during normal operation in the absence of the silicone.

During the same series of plant scale operations, the dimethyl silicone concentrate was added to the tank 21 containing the molten heavy coating asphalt in a proportion to provide one

part per million by volume. Operation with this setup was compared with the operation in the absence of the silicone, and also with a setup in which the same proportion of silicone was added to the coating storage tank 30 following the mixing of the solid filler with the coating asphalt. The presence of entrained vapor bubbles on the coated surface of the travelling sheet persisted in both of the last mentioned operations, whereas with the first mentioned operation in which the silicone was present at the time of mixing the solid filler with the asphalt, entrained bubbles in the coating were practically eliminated. The coated sheet passing to the subsequent sections of the machine was smoother and brighter in appearance than in either of the other two cases.

The following Table I sets forth data obtained during the foregoing operations, with the data in column A representing operation in the absence of added silicone in both the saturating and coating sections, and the data in column B representing operation with added silicone in the saturator and also silicone added to the coating asphalt prior to mixing of the filler there-

with.

Table I

|    | Asphalt Saturant                                           | A      | B      |
|----|------------------------------------------------------------|--------|--------|
| 30 | "Dow-Corning Fluid," P. P. M. by vol.                      | None   | 1      |
|    | Melting point, ball and ring, °F.                          | 119    | 120    |
|    | Penetration at 77° F., ASTM                                | 90     | 92     |
|    | Flash, COC, °F.                                            | 530    | 550    |
|    | Fire, COC, °F.                                             | 630    | 650    |
| 35 | Operating Conditions:                                      |        |        |
|    | Asphalt level in saturator                                 | low    | high   |
|    | Temperature in saturator inlet, °F.                        | 450    | 450    |
|    | Temperature in coating pan, °F.                            | 385    | 390    |
|    | Line speed, ft./min.                                       | 135    | 185    |
|    | Depth of foam in saturator                                 | 4-5'   | 1"     |
| 40 | Tests on Saturated Felt:                                   |        |        |
|    | Per cent voids filled                                      | 86     | 90     |
|    | Per cent saturation                                        | 178    | 199    |
| 40 | Test on Finished Roofing—Accelerated blistering at 225° F. | Severe | Slight |

The foregoing data shows that the very small amount of added silicone has substantially no effect on the physical properties of the asphalt saturant except for an increase in the flash and fire points which is advantageous. Operation in accordance with the present invention gave a saturated felt having 90% of the voids filled with asphalt with a percentage saturation based on the weight of the felt of 199%, representing a substantial improvement over the operation in the absence of the added silicone in the saturant. Moreover, the combination of the treated saturant with the treated coating gave a finished roofing which showed only slight blistering in the conventional accelerated blistering test at 225° F., in comparison to severe blistering for the finished roofing prepared in the absence of the added silicone.

The data in the following Table II illustrates the effect of the saturant consistency on the blistering tendency of roll roofings subjected to atmospheric exposure:

Table II

|                                                           | ASTM Penetration at 77° F.— |
|-----------------------------------------------------------|-----------------------------|
| 70                                                        |                             |
| 6 Months' Atmospheric Exposure                            | 75-90                       |
| No. of roll roofings sampled                              | 47                          |
| Per cent of samples showing severe to moderate blistering | 89.5                        |
|                                                           | 30                          |
|                                                           | 53                          |
|                                                           | 22.5                        |

Thus, of the large number of roll roofings pre-

pared with the conventional asphalt saturant having a penetration of 75-90 at 77° F., 89.5% of these showed severe to moderate blistering after six months' atmospheric exposure. On the other hand, a large number of roll roofings prepared by the same procedure except employing a harder asphalt of about 30 penetration at 77° F. showed greatly improved weatherability, as evidenced by the fact that only 22.5% showed the same degree of blistering after six months' atmospheric exposure.

While the organic silicones have heretofore been proposed as anti-foam additives for organic liquids at atmospheric or mildly elevated temperatures, it could not be foretold in the absence of actual trial that these materials would function to suppress the copious type of foam formed on the surface of the molten asphalt saturant at the high temperatures employed. Moreover, it is considered truly remarkable that the very minute quantity of dispersed silicone within the range specified herein proved capable of handling this severe foaming problem, and at the same time, the desired physical properties of the saturant and the asphalt roofing were not deleteriously affected. Further, the added function of the silicone in providing a heavier surface film of asphalt of characteristic glossy appearance on the surface of the travelling sheet emerging from the saturating bath, which then rapidly dried in during the subsequent cooling period to give substantially improved saturation and percentage of voids filled, was unexpected. Finally, it could not be predicted that the silicone, in the very small proportion employed, would satisfactorily solve the different problem of bubble entrainment in the coating section. The combined steps of the process, as herein described, have resulted in the uniform production of a high quality of asphalt roofing over long periods of continuous operation without difficulty, and without the close attention on the part of the operators as formerly required.

Obviously many modifications and variations of the invention, as hereinbefore set forth, may be made without departing from the spirit and scope thereof, and therefore only such limitations should be imposed as are indicated in the appended claims.

I claim:

1. In the manufacture of asphalt roofing, the method which comprises continuously passing a sheet of felt through a saturating bath of molten normally solid asphalt having an ASTM penetration at 77° F. of about 20-125 maintained at a temperature of 250-450° F. and containing about 0.1-10 parts per million by volume of a liquid dihydrocarbon silicone polymer having anti-foam properties in organic liquids and which is effective to substantially inhibit foaming of said molten asphalt bath, said bath being maintained of sufficient depth and elevated temperature to effectively eliminate moisture from the felt sheet and thoroughly impregnate the same with asphalt, withdrawing the traveling felt sheet from the bath while retaining a substantial surface film of molten asphalt on both sides thereof providing a glossy wet sheet which is then cooled to permit the surface film to rapidly dry in to provide a saturated felt sheet with a minimum of 85% voids filled with asphalt, and then applying a surface coating to the sheet of a mix prepared by adding finely divided solid inorganic filler to previously mixed molten normally solid asphalt and about 0.1-10 parts per

million by volume based on the asphalt of a liquid dihydrocarbon silicone polymer having anti-foam properties in organic liquids and which is sufficient to inhibit entrainment of vapor bubbles in the coating.

5. The method according to claim 1, wherein the asphalt in the saturating bath has an ASTM penetration at 77° F. of about 30-60, and the silicone polymer is present in the saturating bath 10 in the proportion of about 0.1 to 1 part per million by volume based on the asphalt.

15 3. The method according to claim 1, wherein the saturated felt sheet passing to the coating step has a minimum of 87% voids filled with asphalt, and the silicone polymer is present in both the saturating bath and the coating mix in the proportion of about 1 part per million by volume based on the asphalt.

20 4. In the manufacture of asphalt roofing, the steps comprising continuously passing a sheet of felt at a depth of immersion not substantially exceeding about 2½ feet through a presaturating stage of a bath of molten normally solid asphalt having an ASTM penetration at 77° F.

25 25 of about 20-125 maintained at a temperature of 250-450° F. and containing about 0.1-10 parts per million by volume of a liquid dihydrocarbon silicone polymer having anti-foam properties in organic liquids, such operation being effective

30 to vaporize moisture in the felt and provide rapid release of the water vapor from the bath without substantial foaming thereof, removing the felt from the presaturating stage and then passing the felt at a substantially greater depth of immersion more than twice that of the presaturating stage through a saturating stage of the said bath while avoiding the accumulation of a retarding film of vapor on the surface of the immersed sheet to thereby thoroughly impregnate

35 40 the sheet with asphalt, withdrawing the impregnated sheet from the impregnating bath while retaining a substantial surface film of molten asphalt on both sides thereof providing a glossy wet sheet, and finally looping the traveling sheet to provide for cooling and the rapid drying in of the surface film to give a saturated felt sheet with a minimum of 85% voids filled with asphalt.

45 5. The method according to claim 4, wherein the asphalt in the bath has an ASTM penetration at 77° F. of about 30-60, and the silicone polymer is present in the combined presaturating and saturating bath in the proportion of about 0.1 to 1 part per million by volume based

55 on the asphalt.

6. In the manufacture of asphalt roofing, the steps comprising mixing at an elevated temperature finely divided solid inorganic filler with a previously mixed molten normally solid hard 60 coating asphalt and about 0.1-10 parts per million by volume based on the asphalt of a liquid dihydrocarbon silicone polymer having anti-foam properties in organic liquids, and then applying the resultant mix at an elevated temperature as a surface coating to a traveling sheet of asphalt-saturated felt to provide a coating thereon which is substantially free from entrained vapor bubbles.

7. The method according to claim 6, wherein 70 the coating asphalt has an ASTM penetration at 77° F. of about 15-30, the mix is applied at a temperature of about 370-400° F., and the silicone polymer is present in the coating mix in the proportion of about 1 part per million by volume based on the asphalt.

8. The method according to claim 6, wherein the liquid dihydrocarbon silicone polymer is a dimethyl silicone polymer, and is present in the coating asphalt in the proportion of about 1 part per million by volume based on the asphalt.

9. The method according to claim 4, wherein the liquid dihydrocarbon silicone polymer is a dimethyl silicone polymer, and is present in the molten asphalt bath in the proportion of about 1 part per million by volume.

WALLACE A. McMILLAN.

## REFERENCES CITED

The following references are of record in the file of this patent:

## UNITED STATES PATENTS

|    | Number    | Name       | Date           |
|----|-----------|------------|----------------|
| 5  | 1,667,201 | Finley     | Apr. 24, 1928  |
|    | 1,776,586 | Heppes     | Sept. 23, 1930 |
|    | 2,258,218 | Rochow     | Oct. 7, 1941   |
| 10 | 2,322,059 | Roediger   | June 15, 1943  |
|    | 2,350,649 | Speishouse | June 6, 1944   |
|    | 2,375,007 | Larsen     | May 1, 1945    |